

## 1

3,177,093

**METHOD OF TREATING CELLULOSE TEXTILE MATERIAL AND THE TREATED MATERIAL**  
 William Julius van Loo, Jr., Middlesex, and Samuel James O'Brien, Dunellen, N.J., assignors to American Cyanamid Company, Stamford, Conn., a corporation of Maine

No Drawing. Continuation of application Ser. No. 796,209, Mar. 2, 1959. This application June 6, 1962, Ser. No. 200,315

10 Claims. (Cl. 117—139.4)

The present invention relates to the method of applying thermosetting cyclic urea-formaldehyde resins to cellulose-containing textile materials, and to the materials so treated, and more particularly to a method for obtaining higher than normal tensile strength on cellulose-containing textile materials with little or no sacrifice in wrinkle recovery.

In the past, the textile industry has employed many finishes of the resin type to impart wrinkle resistance and dimensional stability to cellulosic materials, such as cotton, viscose rayon and the like. One of the first of these resins to be used was the urea-formaldehyde type. This product had serious defects in that it caused extensive tensile strength losses when the amount of resin applied was sufficient to give satisfactory crease resistance. This was particularly true when used on cotton fabrics. In addition, the loss in tensile strength when a fabric was scorched after chlorine bleaching was extensive.

Gradually, the urea-formaldehyde resin was replaced with the methylated methylol melamine resins, which imparted satisfactory crease resistance to cellulose textile materials at lower concentrations and without serious loss in tensile strength due to chlorine belaching. However, during use, it was discovered that certain methylated methylol melamines had the somewhat serious defect of discoloring when the fabrics were subjected to a bleaching operation in which chlorine was used.

In order to avoid the disadvantages of yellowing following chlorine bleaching which resulted when some methylated methylol melamine resins were used, recourse was had to the use of ethylene urea type resins. These materials had the advantage that they did not discolor fabric treated therewith after bleaching with chlorine and further that they could be used in high concentrations to obtain excellent high wrinkle recovery without imparting stiffness to the fabrics. The ethylene urea or cyclic urea type resin, however, had the disadvantage that they gave a substantially greater loss in tensile strength than the methylated melamine resins when fabrics treated therewith were subjected to scorching after chlorine bleaching.

Aside from these special considerations, in general, it may be stated with respect to most thermosetting textile resin finishes, that as resin solid on the fabric increases and wrinkle recovery increases, the tensile strength of the finished textile material is adversely affected, and in general declines. Thus, the problem of maintaining a high wrinkle recovery without adversely affecting the tensile strength of the finished fabric has presented a genuine challenge to the textile finishing industry.

Accordingly, it is an object of the present invention to provide a process whereby a wrinkle resistance of high order may be achieved, while simultaneously maintaining a high order of tensile strength.

It is a further object of the present invention to provide such a process which may be readily and economically adapted by most textile finishing installations.

These and other objects and advantages of the present invention will become more apparent from the detailed description thereof set forth hereinbelow.

## 2

In accordance with the present invention a method is provided for the treating of cellulose-containing textile materials whereby a high order of tensile strength and wrinkle recovery are obtained even at high resin solids on the fabric, which comprises applying thereto a formaldehyde condensate of a cyclic urea, and thereafter curing said cyclic urea in the presence of a zinc salt catalyst in an atmosphere of steam. Following the effective curing of the above described conditions, the so finished fabric is allowed to dry, either at room temperature or under the normal drying conditions employed in textile finishing plants.

By the expression "formaldehyde condensates of cyclic ureas," as that term is employed herein, we refer to the methylol derivatives, of ethylene urea and certain of its homologs, as for example, 1,2-propylene urea, and certain alkyl substituted derivatives thereof, as well as hydroxyl substituted derivatives thereof.

In general, these compounds may be characterized by the following general formula:



wherein R<sub>1</sub> through R<sub>4</sub> are selected from the group consisting of hydrogen, saturated aliphatic alkyl groups containing from 1 to 4 carbon atoms, and hydroxyl. The preferred species within the above general formula is where R<sub>1</sub> through R<sub>4</sub> is hydrogen or where one of the values is methyl and the remainder are hydrogen. With respect to alkyl substitution for R<sub>1</sub> through R<sub>4</sub>, the total number of carbon atoms in substituting groups should not exceed 6.

While in the above general formula, the dimethylol derivative is illustrated, it should be noted that while the dimethylol derivative is preferred, cyclic ureas having at least 1.5 mole of combined formaldehyde as methylol formaldehyde are fully contemplated in accordance with the present invention.

The cyclic ureas which are condensed with formaldehyde to form methylol derivatives employable in the process of the present invention may be prepared in accordance with known prior art procedures by reacting a suitable diamine, including the substituted diamines, with urea, as for example, in accordance with the procedures described in U.S. Patents Nos. 2,436,311 and 2,517,750, which are incorporated herein by reference. As examples of suitable 5-membered cyclic ureas within the purview of the present invention, the following are illustrative:

- 2-imidazolidinone (ethylene urea);
- 3-methyl-2-imidazolidinone, 1,2-propylene urea;
- 3,4-dimethyl-2-imidazolidinone;
- 3,3,4-trimethyl-2-imidazolidinone;
- 3,3,4,4-tetramethyl-2-imidazolidinone;
- 3,4-diethyl-2-imidazolidinone;
- 3,3-dimethyl-4-ethyl-2-imidazolidinone;
- 3-methyl-3-ethyl-2-imidazolidinone;
- 3,4-dimethyl-3-n-propyl-2-imidazolidinone;
- 3-isopropyl-2-imidazolidinone;
- 3-methyl-3-isopropyl-4-ethyl-2-imidazolidinone;
- 3-n-butyl-2-imidazolidinone;
- 3-ethyl-4-sec-butyl-2-imidazolidinone;
- 3-hydroxy-2-imidazolidinone;
- 3,4-dihydroxy-2-imidazolidinone;
- 3-hydroxy-4-methyl-2-imidazolidinone;
- 3,4-dihydroxy-3,4-dimethyl-2-imidazolidinone;
- 3-hydroxy-3-methyl-4-n-propyl-2-imidazolidinone; and
- 3-hydroxy-3-ethyl-4-methyl-4-isopropyl-2-imidazolidinone.

The above identified cyclic ureas and their equivalents are condensed with formaldehyde or methylolated in accordance with known prior art techniques for methylolating aminoplast resins with formaldehyde. The term "formaldehyde" as it is employed herein, refers to formaldehyde per se, including formalin solutions or para-formaldehyde or formaldehyde engendering substances, such as hexamethylenetetramine, glyoxal, and the like. In general, the cyclic urea is reacted in an aqueous medium in a mole ratio of from one mole of the ureas to from one to three moles of the formaldehyde and preferably with from two to three moles of formaldehyde. The methylolation may be carried out at a pH of from between 3 and 10 and preferably at a pH of from between 7 and 10 at a temperature of from between 40° and reflux or about 100° C. until solution is achieved. Thereafter, the reaction mixture is cooled. Preferably, the mole ratio between the cyclic urea and formaldehyde is 1 to 2, respectively. When the formaldehyde is increased, the degree of methylolation is not appreciably increased and the presence of increased amounts of free formaldehyde increases handling difficulties and presents other known problems. When the mole ratio is 1 to 2, the resulting product may be identified as a dimethylol compound in that by analysis, as much as 1.9 moles of the available 2 moles of formaldehyde are combined.

As indicated hereinabove, the present invention is applicable to textile materials containing cellulose. The term "cellulose textile material" and similar expressions as they are employed herein, is intended to include textile materials including fibers, filaments, yarns, formed fabrics, containing at least 50% cellulose. Materials, as for example, flax, cotton, jute, hemp, sisal, and regenerated cellulose, as for example, viscose rayon, cuprammonium or the like are also included. In its more preferred sense, expressions such as are identified above and similar expressions, are intended to include cotton and viscose rayon textile fabrics, whether they be woven, knitted, non-woven, felted or otherwise formed.

The methylol condensates of cyclic ureas as they are identified hereinabove may be applied to textile materials in amounts varying between 1 to 40%, based on the dry weight of the material, and preferably in amounts of from between 2.5 and 25% by weight. These heat-curable resinous materials may be applied by padding, dipping, spraying, immersion or other suitable techniques, but are preferably applied by conventional padding processes, as in the case of formed fabrics, in that most textile finishing installations are equipped for such applications.

It is a unique characteristic of the present process that the ureas in accordance with this invention and the unexpected results obtained therefrom are only realized when the resin is cured in the presence of zinc salts as curing accelerators or catalysts. Thus, for example, most of the better known curing accelerators presently employed in the textile finishing industry, such as various metal salts, prominent among which are magnesium chloride, aluminum chloride, ammonium salts, such as ammonium chloride, amine salts, such as triethylamine hydrochloride, alkanol amine salts, such as triethanolamine hydrochloride, and free acids, such as oxalic, tartaric, and the like, are not applicable in accordance with the present process. As noted, the only catalysts that we have found to be suitable in accordance with our present invention are inorganic salts of zinc. "Zinc salts" as that term is employed herein, is intended to include the salts derived from the reaction of zinc oxide or zinc hydroxide with inorganic acids. Thus, for example, the expression includes zinc chloride, zinc sulfate, zinc nitrate, and the like. Of these enumerated, zinc nitrate is greatly preferred because of its solubility and pad bath stability. In general, zinc catalysts are employed in amounts of from between 1 and 36%, based on the weight of resin solids employed

in accordance with the present procedure and more preferably in amounts of from between 5 and 15%, based on the weight of resin solids employed in a given treating solution.

In addition to the present invention being limited to cyclic urea resins and zinc salt curing accelerators in order to achieve unexpected properties, it is essential that curing be accomplished in an atmosphere of steam so that in effect the cure is accomplished when the finished material is in the wet state. Although an atmosphere of steam at approximately 212° F. is recommended for the curing process, the temperature of the steam may vary from between 80° F. to about 250° F. or even higher. The higher the temperature values being achieved by employing super-atmospheric pressure while curing in a steam atmosphere below about 212° F. is readily accomplished by curing at sub-atmospheric pressures. In general, longer time cycles are required at the lower temperatures and shorter cycles for the higher temperatures. Although curing in an atmosphere of steam is greatly preferred, the curing may be accomplished in the absence of added steam and only that steam which is generated through the drying of the impregnated fabric need be employed. Normally, this may be accomplished by placing the treated material prior to cure in a substantially (almost completely) closed container or chamber. Additionally, a partially saturated atmosphere of steam may be employed. A confined or unconfined atmosphere may be used.

In general, curing times employed in the present process are somewhat longer than those conventionally used. Thus, in general, times from about 15 minutes to about 3 hours are employed to best advantages. While the time of cure may be shortened or lengthened within given limits depending upon other variables such as steam temperature, amount of catalysts, etc., it is usually preferred to effect cure at times between about 30 minutes and 2½ hours.

In order to illustrate the present invention, the following examples are given by way of illustration. No details or enumerations contained therein should be construed as limitations on the present invention, except insofar as they appear in the appended claims. All parts and percentages are by weight unless otherwise indicated.

#### EXAMPLE 1

Pad baths were prepared containing 19.0%, 27.5% and 35.0% resin solids of dimethylol ethylene urea and 12% on the weight of the resin solids in the bath of zinc nitrate or magnesium chloride as curing accelerators.

16.1%, 23.4% and 29.6% applications of dimethylol ethylene urea were made on 80 x 80 cotton percale by padding with the above solutions, using a pick-up of 85%.

Two methods of curing were used:

A. Dried at 225° F. for 2 minutes and then heated at 350° F. for 1.5 minutes by the standard procedure.

B. The wet fabric was rolled and placed in a test tube having a small vent for escape of pressure. The test tube and fabric were then heated in an oven for 2.5 hours. The damp fabrics were then dried at room temperature.

The treated fabrics were analyzed for nitrogen, before and after washing for 30 minutes in boiling water followed by a water rinse and drying at room temperature.

The wrinkle recovery was measured on a Monsanto Wrinkle Recovery Tester following the tentative Test Method 66-1956 described on page 158 of the 1957 Technical Manual and Year Book of the American Association of Textile Chemists and Colorists, vol. 33. The tensile strength was measured on a Scott Tester according to A.S.T.M. standards and the values reported are in pounds.

The results of these applications are shown in Table I below.

Table I

| Percent Resin on Fabric | Catalyst                          | Curing Conditions | Percent Nitrogen |        | Tensile Strength, Pounds | Wrinkle Recovery Total |
|-------------------------|-----------------------------------|-------------------|------------------|--------|--------------------------|------------------------|
|                         |                                   |                   | Orig.            | Washes |                          |                        |
| 16.1                    | Zn(NO <sub>3</sub> ) <sub>2</sub> | A                 | 2.7              | 2.2    | 52                       | 290 <sup>a</sup>       |
| 16.1                    | Zn(NO <sub>3</sub> ) <sub>2</sub> | B                 | 2.5              | 1.7    | 74                       | 285                    |
| 23.4                    | Zn(NO <sub>3</sub> ) <sub>2</sub> | A                 | 3.7              | 2.4    | 57                       | 311                    |
| 23.4                    | Zn(NO <sub>3</sub> ) <sub>2</sub> | B                 | 3.5              | 2.2    | 73                       | 293                    |
| 23.4                    | MgCl <sub>2</sub>                 | A                 | 3.3              | 2.6    | 52                       | 291                    |
| 23.4                    | MgCl <sub>2</sub>                 | B                 | 3.1              | 0.6    | 94                       | 223                    |
| 29.6                    | Zn(NO <sub>3</sub> ) <sub>2</sub> | A                 | 4.2              | 2.6    | 58                       | 297                    |
| 29.6                    | Zn(NO <sub>3</sub> ) <sub>2</sub> | B                 | 4.9              | 2.5    | 77                       | 285                    |
| 29.6                    | MgCl <sub>2</sub>                 | A                 | 4.0              | 2.6    | 52                       | 295                    |
| 29.6                    | MgCl <sub>2</sub>                 | B                 | 3.7              | 0.6    | 94                       | 226                    |

The following conclusions may be drawn from these 20 results:

(1) Dimethylol ethylene urea can be cured on the fabric at 210° F. (in steam) with zinc nitrate as a catalyst to obtain approximately normal wrinkle recovery and higher than normal tensile strength. Good fixation of 25 resin is obtained, as indicated by the nitrogen analysis.

(2) Curing under the same conditions with magnesium chloride as the catalyst gives poor fixation of the resin and lower than normal wrinkle recovery.

In addition, Table I hereinabove clearly illustrates the 30 merit of the present invention, in that as will be seen the conditions of the present process result in wrinkle recoveries substantially as good as are those obtained under normal curing conditions, but with tensile strengths of the order of at least about 70 pounds, which is considerably higher than that normally obtained when wrinkle recovery values of this magnitude are obtained. This tensile strength is of the order of 20 pounds higher than normally obtained for wrinkle recoveries of this magnitude. In general, it has been found that tensile strength values of the order of at least 80 pounds may be achieved for wrinkle recoveries of 240° and higher, and that for wrinkle recoveries higher than 280° tensile strengths of the order of greater than about 70 pounds are readily achieved by employment of the present process. Such values heretofore have not been possible.

## EXAMPLE 2

In separate applications, 17.65% of dimethylol ethylene urea was applied to cotton percale employing varying amounts of well known curing accelerators, based on the weight of resin solids. An 85% wet pick-up was obtained, leaving 15% resin solids on the weight of the fabric. The fabric was then steam cured for 2.5 hours at 210° F. The applied solutions were as follows.

All solutions contained 17.65% dimethylol ethylene urea.

- A. 3.5% ammonium sulfate.
- B. 7.0% 2-methyl-2-amino-propanol-1-hydrochloride.
- C. 7.0% pyridine hydrochloride.
- D. 0.5% oxalic acid.

The results of the applications according to Example 2 are set forth in Table II below.

Table II

| Treatment: | Wrinkle recovery (total W+F) |
|------------|------------------------------|
| A          | 175                          |
| B          | 165                          |
| C          | 172                          |
| D          | 185                          |
| Untreated  | 150                          |

No tensile strength determinations were made since they were not warranted in view of the wrinkle recovery obtained employing these known catalysts. Table II fur-

ther illustrates the unique character of zinc salts in the present invention. Compare with Example 1.

## EXAMPLE 3

In separate applications, solutions containing 9.4, 13.5 and 17.65% solids of dimethylol melamine and of dimethylol ether of trimethylol melamine were applied to cotton percale. The solutions contained 12% of either magnesium chloride or zinc nitrate based on the weight of resin solids as catalyst. An 85% wet pick-up was obtained in all cases, leaving the solids content indicated in Table III below on the fabric. The cures identified as A and B in said table are the same as those described in Example 1 hereinabove.

Table III

| Resin                                  | Solid (OWF) | Wrinkle Recovery MgCl <sub>2</sub> Cure |     | (Total W+F) Zn(NO <sub>3</sub> ) <sub>2</sub> Cure |     |
|----------------------------------------|-------------|-----------------------------------------|-----|----------------------------------------------------|-----|
|                                        |             | A                                       | B   | A                                                  | B   |
| Dimethylol melamine                    | 8           | 235                                     | 163 | 239                                                | 199 |
|                                        | 11.5        | 244                                     | 169 | 259                                                | 210 |
| Dimethyl ether of trimethylol melamine | 15.0        | 243                                     | 170 | 269                                                | 230 |
|                                        | 8           | 248                                     | 163 | 255                                                | 183 |
|                                        | 11.5        | 244                                     | 169 | 266                                                | 202 |
|                                        | 15.0        | 243                                     | 170 | 261                                                | 201 |

No tensile strength determinations were made since they 45 were not warranted in view of the wrinkle recovery obtained. Table IV illustrates the unique character of the cyclic ureas in the present invention. Compare Examples 1 and 3.

## EXAMPLE 4

In separate applications, solutions containing 24.9 and 32.5% (solids basis) of the dimethyl ether of dimethylol urea (UF) was applied to cotton percale employing 12%, based on resin solids, of either magnesium chloride or zinc nitrate as catalyst. An 85% wet pick-up was obtained and the finished fabric cured by the cures identified as A and B in Examples 1 and 2 above. The results are recorded in Table IV below.

Table IV

| UF Solids | MgCl <sub>2</sub> |    |        |    | Zn(NO <sub>3</sub> ) <sub>2</sub> |    |        |    |
|-----------|-------------------|----|--------|----|-----------------------------------|----|--------|----|
|           | Cure A            |    | Cure B |    | Cure A                            |    | Cure B |    |
|           | WR                | TS | WR     | TS | WR                                | TS | WR     | TS |
| 21.2      | 238               |    | 179    |    | 264                               | 56 | 264    | 62 |
| 27.6      | 240               |    | 190    |    | 228                               | 69 | 271    | 60 |

In Table IV above, tensile strength determinations for 70 fabrics having a urea-formaldehyde resin thereon cured with magnesium chloride were deemed unwarranted, since the wrinkle recovery obtained by steam cure was not satisfactory. While good wrinkle recovery can be obtained employing urea-formaldehyde resins by steam cur-

ing where a zinc salt is the catalyst, no significant advantage in tensile strength is obtained with respect to those achieved by conventional cure. The present table further demonstrates that the advantages of the present invention are for the most part limited to cyclic ureas of the type contemplated by the present invention.

While the present invention has been described specifically with respect to the methylol condensates of 5-ring membered cyclic ureas, it is to be understood that the term as it is employed hereinabove is intended to include their alkylated and in particular their methylated derivatives. Since alkylation and particularly methylation are, in general, employed to stabilize aminoplast resins, alkylations of the condensates contemplated in accordance with the present invention are in general unnecessary, in that these materials are themselves sufficiently stable. However, should alkylation or methylation be desired, this may be carried out in accordance with the prior art procedures known for the methylation of aminoplast resins.

Any of the cyclic ureas identified hereinabove or catalysts set forth therein suitable for use in the present invention may be employed singly or in combination with one another, and to some extent with other known textile finishing resins, as for example, urea-formaldehyde resins and their alkylated derivatives, melamine-formaldehyde resins and their alkylated derivatives, 6-ring membered cyclic ureas, such as 1,3-propylene urea-formaldehyde condensates and derivatives thereof, epoxy resins, such as the diglycidyl ether of ethylene glycol, diglycidyl ether per se and the like guanamine-formaldehyde resins and their alkylated derivatives, acetone-formaldehyde resins and other known textile finishing resins wherein their incorporation with the cyclic ureas in accordance with the present invention does not significantly affect the properties sought to be achieved.

In addition, it will be apparent that other textile finishing assistants may be employed in the process of the present invention, such as wetting agents, softeners and the like, insofar as their inclusion in the treating bath in no way significantly impairs the effect sought to be achieved.

This application is a continuation application of application Serial No. 796,209, filed March 2, 1959, now abandoned.

We claim:

1. A method of treating cellulose textile material whereby high tensile strength and wrinkle recovery are obtained, which comprises applying thereto, from an aqueous solution, a formaldehyde condensate of a 5-membered cyclic urea and a zinc salt of an inorganic acid as a catalyst therefor, and immediately, without intermediate drying, wet curing said cyclic urea in an atmosphere of

wet steam, maintaining the textile material in the wet state until completion of the cure and thereafter drying the fabric.

2. A method according to claim 1, wherein the amount of resin applied is from between 1 to about 40%, based on the weight of the textile material.

3. A method according to claim 1, wherein the amount of zinc salt catalyst is from between 1 and 36%, based on the weight of resin solids.

4. A method according to claim 1 wherein the catalyst is zinc nitrate.

5. A process according to claim 1, wherein the cyclic urea is ethylene urea.

6. A process according to claim 1, wherein the cyclic urea is 1,2-propylene urea.

7. A process according to claim 1, wherein the curing takes place at a temperature of from between about 80° F. to about 250° F.

8. A cellulose containing material prepared by the process of claim 1 having from 1 to 40% based on the weight of the textile material, of a water-soluble cured formaldehyde condensate of a 5-membered cyclic urea thereon and characterized by high tensile strength and wrinkle recovery.

9. A cotton textile material prepared by the process of claim 1 having from 1 to 40% based on the weight of the textile material of a cured formaldehyde condensate of ethylene urea thereon.

10. A method for treating formed cotton fabric whereby high tensile strength and wrinkle recovery are obtained, which comprises applying from an aqueous solution from about 2.5 to about 25% of a formaldehyde condensate of a 5-membered cyclic urea and a zinc salt of an inorganic acid as a catalyst therefor, said zinc salt being selected from the group consisting of zinc chloride, zinc sulfate and zinc nitrate, and immediately, without intermediate drying, wet curing said cyclic urea in the presence of said zinc salt catalyst in an atmosphere of wet steam and thereafter drying the so-processed cotton fabric.

#### References Cited by the Examiner

##### UNITED STATES PATENTS

|           |       |                  |       |              |
|-----------|-------|------------------|-------|--------------|
| 2,088,227 | 7/37  | Battye et al.    | ----- | 117—139.4    |
| 2,254,001 | 8/41  | Conway.          |       |              |
| 2,661,312 | 12/53 | Richardson       | ----- | 117—139.4    |
| 2,763,574 | 9/56  | Ruperti          | ----- | 117—138.5    |
| 2,899,263 | 8/59  | Nuessle et al.   | ----- | 117—139.4 XR |
| 2,917,412 | 12/59 | Reinhardt et al. | ----- | 117—139.4    |
| 2,974,065 | 4/61  | Mann et al.      | ----- | 117—145 XR   |

WILLIAM D. MARTIN, Primary Examiner.

RICHARD D. NEVIUS, Examiner.

UNITED STATES PATENT OFFICE  
CERTIFICATE OF CORRECTION

Patent No. 3,177,093

April 6, 1965

William Julius van Loo, Jr., et al.

It is hereby certified that error appears in the above numbered patent requiring correction and that the said Letters Patent should read as corrected below.

Column 1, line 34, for "belaching" read -- bleaching --; column 2, line 15, strike out the comma; column 3, line 10, for "ureas" read -- urea --; line 34, for "cuprammonium" read -- cuprammonium rayon --; column 4, line 38, for "catalysts" read -- catalyst --; column 7, line 31, after "like" insert a comma.

Signed and sealed this 5th day of October 1965.

(SEAL)

Attest:

ERNEST W. SWIDER  
Attesting Officer

EDWARD J. BRENNER  
Commissioner of Patents